

## UNITED STATES PATENT OFFICE

THOMAS H. STACKHOUSE, OF WILMINGTON, DELAWARE

## MOTOR FUEL

No Drawing.

Application filed November 25, 1925. Serial No. 71,436.

The object of my invention is to provide a motor fuel having anti-knock qualities. More specifically stated, the object of the invention is to utilize gasoline as the main constituent of the motor fuel and add thereto a material which, without perceptibly impairing any known quality of gasoline that contributes to its efficiency as a motor fuel, will impart to it the anti-knock qualities desired. To produce a commercially practicable result, several requirements must be met. The material added must be in a very small proportion, inasmuch as a reduction of the amount of gasoline in a gallon of the composite fuel will to that extent rob the gasoline of those desirable qualities which it is desired to preserve. The added material must be so relatively inexpensive that it will not add more than a small fraction of one cent to the cost of the gasoline, in order that the composite fuel may be retailed at the same price as ordinary gasoline, or at least so that an increase of less than one cent per gallon in the wholesale price will yield a substantially larger profit to the refiner. The added material should be readily and permanently soluble in the gasoline, at all ordinary temperatures, without the necessity of special agitation or of any other special mixing process that would perceptibly add to the cost of production of commercial gasoline.

The above results are accomplished by the addition to gasoline of from one-fourth of one per cent to two per cent of carbon bisulfide with the preferential addition of nitrobenzene in an amount not over three per cent of the carbon bisulfide. The nitrobenzene is preferably added to the carbon bisulfide before the latter is added to the gasoline. The nitrobenzene may be omitted altogether, but its addition, besides assisting in the attainment of the result sought and securing the result sought with more certainty, reduces the amount of carbon bisulfide required by an amount exceeding the amount of carbon bisulfide that it displaces.

Gasoline itself is so variable with respect to the degree to which it approaches the desideratum of avoiding knocking in an ordinary internal combustion engine, that it is

impossible to specify the proportion of carbon bisulfide to be added to the gasoline within a range narrower than that above given. Thus, the combustion of gasoline that is obtained from the crude oil by topping, or ordinary distillation at atmospheric pressure, will ordinarily produce more knocking than will the combustion of gasoline that is manufactured from higher boiling point constituents of crude oil by cracking. Then, too, gasoline produced from crude petroleums of different origins will have substantially different qualities. With the average gasoline, the addition of from one-half to one per cent of carbon bisulfide will produce an anti-knock motor fuel.

The addition of one-half of one per cent of pure or refined carbon bisulfide to gasoline will not increase the cost of the fuel over that of simple gasoline by more than about one-tenth of one cent per gallon.

The carbon bisulfide should be approximately pure, that is approximately 99.9% pure, and should be almost or quite without free sulfur, although a somewhat lower degree of purity, while undesirable, is efficient.

It is preferred to add the carbon bisulfide, or the solution of carbon bisulfide and nitrobenzene, to a little gasoline before the addition to the body of gasoline which it is desired to convert into an anti-knock motor fuel. This is especially desirable where the material is to be sold in the open market for addition to ordinary commercial gasoline. The proportion of the gasoline-carbon bisulfide solution that is added to the commercial gasoline will of course vary with the proportion of gasoline in the solution to be added.

The main reason for the effectiveness of my improved motor fuel is that the combustion, instead of being nearly instantaneous, is progressive, that is, combustion continues substantially throughout the stroke of the piston and is completed near or at the end of its stroke. The result is substantially higher efficiency and greater power with elimination of knocking. Another important advantage that is attained by progressive combustion is the substantial prevention of formation of

carbon or the substantial elimination of any carbon that may be formed and deposited.

It is clear, from the foregoing explanation, that any negligible increase in the cost of the improved fuel over that of straight gasoline is compensated, many times over, by the saving in cost due to increased efficiency and power.

While I have specified "gasoline" as the main ingredient of my improved motor fuel, it will be understood that "gasoline" is a somewhat flexible term which, in the progress of the art, has come to be applied to what, in earlier years, was known commercially as high-grade kerosene. Therefore, it is to be understood that by specifying gasoline I mean to include as an equivalent any grade of kerosene that, now or in the future development of the art, may be substituted for gasoline as a motor fuel.

While I have specified upper and lower limits, workable and preferential, for the proportion of carbon bisulfide, that proportion could be increased somewhat above the one or two per cent specified, without detriment, but without advantage. I, therefore, do not wish to limit myself to the maximum proportion of carbon bisulfide specified. However, if the proportion of carbon bisulfide should be increased to beyond (say) five, or, at the most, ten per cent, its use would probably be detrimental, not merely in that it would reduce the efficiency of the gasoline by reducing the proportion of gasoline, but also in that it would be apt to produce deleterious effects on the metal with which the fuel comes into contact.

In place of nitrobenzene I may use such equivalent substances as nitrotoluol and nitroxyol and perhaps other nitrocarbons.

The percentage may be increased beyond three per cent of the carbon bisulfide without detriment but without advantage.

Having now fully described my invention, what I claim and desire to protect by Letters Patent is:

1. An anti-knock motor fuel comprising a solution of gasoline, carbon bisulfide and nitrobenzene, the gasoline comprising a predominating proportion of the composition and the proportion of carbon bisulfide greatly exceeding the proportion of nitrobenzene.

2. An anti-knock motor fuel comprising a solution of gasoline, carbon bisulfide and nitrobenzene, the carbon bisulfide comprising between over one-fourth of one per cent and less than five per cent of the solution and the proportion of nitrobenzene being very much less than that of the carbon bisulfide.

In testimony of which invention, I have hereunto set my hand at Philadelphia, Penna., on this 5th day of November, 1925.

THOMAS H. STACKHOUSE.